

## UNITED STATES PATENT OFFICE

FRITZ ROTHE AND HANS BRENEK, OF BERLIN, GERMANY, ASSIGNEES TO THE FIRM  
RHENANIA-KUNHEIM VEREIN CHEMISCHER FABRIKEN A. G., OF BERLIN, GERMANY

PROCESS FOR OBTAINING BARIUM-ORTHO-SILICATE OR BARIUM-TRI-SILICATE BY  
THE DECOMPOSITION OF BARIUM CARBONATE

No Drawing. Application filed May 27, 1927, Serial No. 194,854, and in Germany August 27, 1926.

The invention has reference to a process for obtaining bariumorthosilicate or bariumtrisilicate and more particularly to an improvement of the known process consisting in burning a mixture of bariumcarbonate together with silica or bariummetasilicate at a temperature of 1400-1500° centigrade.

The object of this invention is to improve this method in order to decrease the temperature required for this reaction. We have found that it is possible to lower the temperature at which said reaction takes place, by carrying out the heating process in the presence of steam. In this manner it is possible to lower the temperature to about 1000-1100° centigrade.

The process may be carried out in a revolving tube furnace, and it is of special importance that the heating gases contain a sufficient quantity of steam to act upon the mixture of barium carbonate and silica containing material during the burning operation. It is possible either to add the steam to the heating gases or to utilize for heating the furnace fuels which contain sufficient quantities of hydrogen which is formed into steam at their combustion. Oil, producer gas from lignite, water gas or the like may be used for this purpose.

The bariumorthosilicate or bariumtrisilicate obtained by this process may be transferred, for instance by a treatment with water, into barium hydroxide, the rest of BaO remaining bound to silica in the form of barium metasilicate. It is of special advantage to utilize said barium metasilicate to act upon the bariumcarbonate. In this manner the silica can be used for several times for the reaction and consequently any sulphur compounds or sulphuric salts which may be formed during the operation or may be contained in the barium carbonate, are expelled, so that the products obtained are free from sulphur.

The following examples show that the presence of steam has really the important effect above explained.

(1). A mixture of 100 parts of a pure barium carbonate and 15.6 parts of sand with 50 98% of  $\text{SiO}_2$  are burnt for two hours in the

presence of heating gases having 15% by volume of steam at a temperature of 1100° centigrade. The loss of glowing amounts to 24.47%. If a complete formation of orthosilicate would have taken place, half of the content of BaO, that is 41% of the weight of the glowing product must go in solution on lixiviation, whereas the other half thereof remains as barium metasilicate and goes in solution only upon a treatment with hydrochloric acid. On lixiviating with water the heating produced obtained in the above described manner, 39% of its weight is ascertained as BaO soluble in water, whereas 41% of its weight consists of BaO only soluble in hydrochloric acid. Thus the barium carbonate is completely transferred into barium orthosilicate by heating it together with sand, in the presence of steam at 1100° centigrade.

(2). The same mixture renders, if heated at 1200° centigrade without the presence of steam during two hours, however, only 21.8% of water soluble BaO and only after heating during two hours at 1450° centigrade 38.2% of water soluble BaO can be obtained.

The results of these examples show that by heating in the presence of steam a complete transformation of barium carbonate into orthosilicate is possible at a relatively low temperature. Consequently the described process renders the considerable advantage, that on the one hand the want of fuel is essentially lowered and on the other hand the furnace lining is saved.

It will be understood that when in this specification and the appended claims we speak of "silica containing material" we mean to include pure silica.

What I claim and desire to secure by Letters Patent of the United States is:

1. The process for obtaining bariumorthosilicate or bariumtrisilicate by the decomposition of barium carbonate comprising heating barium carbonate together with silica containing material in the presence of steam.

2. The process for obtaining barium orthosilicate or barium trisilicate by the decomposition of barium carbonate comprising heating barium carbonate together with 100

barium metasilicate in the presence of steam.

3. The process for obtaining barium orthosilicate or barium trisilicate by the decomposition of barium carbonate comprising heating barium carbonate in the presence of steam together with barium metasilicate which is obtained from the barium silicate formed by the reaction of barium carbonate and silica.

10 4. The process for obtaining barium orthosilicate or barium trisilicate by the decomposition of barium carbonate comprising heating barium carbonate together with silica containing material in the presence of 15 steam at a relatively low temperature.

5. The process for obtaining barium orthosilicate or barium trisilicate by the decomposition of barium carbonate comprising heating barium carbonate together with 20 silica containing material in the presence of steam at about 1000-1100° centigrade.

6. The process for obtaining barium orthosilicate or barium trisilicate by the decomposition of barium carbonate comprising 25 heating barium carbonate together with silica containing material in the presence of steam by the aid of fuels rich in hydrogen, which form vapour at their combustion.

7. The process for obtaining barium orthosilicate or barium trisilicate by the decomposition of barium carbonate comprising heating barium carbonate together with silica containing material, heating gases having 30 15% by volume of steam being present during the heating operation to act upon the mixture.

FRITZ ROTHE  
HANS BRENEK.

40

45

50

55

60

65